

# United States Patent

[11] 3,625,878

[72] Inventors **Henri Gourlaouen**  
Mont-Saint-Aignan;  
**Christian Jahan, Bois-Guillaume; Robert**  
Muths, Mont-Saint-Aignan; **Jean**  
Taillardat, Mont-Saint-Aignan, all of  
France  
[21] Appl. No. **885,970**  
[22] Filed **Dec. 17, 1969**  
[45] Patented **Dec. 7, 1971**  
[73] Assignee **Esso Research and Engineering Company**  
[32] Priority **Dec. 30, 1968**  
[33] **France**  
[31] **181618**

[54] **OXIDATION-RESISTANT MINERAL OIL**  
19 Claims, No Drawings

[52] U.S. Cl..... **208/14,**  
208/264, 252/63

[51] Int. Cl..... **H01b 3/22**  
[50] Field of Search..... **208/14, 19;**  
**252/63**

[56] **References Cited**  
UNITED STATES PATENTS

3,318,799 5/1967 Acker et al. .... **208/14**

*Primary Examiner*—Herbert Levine  
*Attorneys*—Pearlman and Stahl and Frank T. Johmann

**ABSTRACT:** A stable mineral oil composition comprises a base mineral oil to which has been added a synergistically acting mixture of heavy cycle gas oil and coal oil obtained from the distillation of coal tars. Preferably, at least one of the components of the composition has been subjected to mild hydrogenation.

## OXIDATION-RESISTANT MINERAL OIL

The present invention relates to mineral oils which are resistant to oxidation, and to a process for making such mineral oils, and in particular, although not exclusively, the invention relates to such mineral oils which contain a significant proportion of aromatic compounds, which thereby gives them a high degree of utility as electrical oils.

It is well known that insulating oils have to perform very long-term service in electrical apparatus. It is therefore particularly important that these oils should withstand oxidation well. The oils prepared by the usual refining processes withstand oxidation better the closer their content of aromatic compounds is to an optimum value, which is relatively low. Nevertheless, the insulating oils which, in modern electrical apparatus, are subjected to ever higher electrical fields, must not only possess exceptional stability, but also have the property of dissolving any gases which may be liberated and form dangerous pockets in high-tension apparatus. This latter requirement is at present incompatible with the previous one, since the oils absorb the liberated gases better the more aromatic they are.

It is already known that the resistance of oils to oxidation is improved by adding to them, in the course of refining, a small quantity of a petroleum fraction known in the trade as "heavy cycle gas oil." Heavy cycle gas oil will hereinafter be designated H.C.G.O. and is a distillation fraction of heavy products that are formed, at the same time as light products, in cracking operations, such as catalytic cracking operations, for instance.

The oils to which the H.C.G.O. is added are usually mineral oils prepared by refining petroleum distillates or deasphalted residues according to processes comprising various treatments, the most usual of which are treatment by a selective solvent such as phenol or furfural to remove at least some of the aromatic compounds, dewaxing, treatment by sulfuric acid or oleum, treatment by an activated earth and for hydrogenation. The refining process is selected according to the nature of the crude and in accordance with the uses to which the oil is to be put, as required.

The H.C.G.O. is very rich in aromatic and heteroaromatic compounds. To the mineral oils are added about 4 percent by weight of H.C.G.O. The aromatic character of the oil is thus enhanced, but the benefits of this increase in aromaticity are limited, for beyond the proportion of 4 percent, which corresponds to an optimum, the incorporation of an additional quantity of H.C.G.O. does not favorably influence the stability of the resulting oil blend.

It is also known that the stability of mineral oils can be improved by the addition, in the course of refining, of a small quantity of a coal oil, as for instance, an anthracene or a chrysene oil, which oils are characterized by a high content of aromatic and heteroaromatic compounds. The optimum proportion is between 0.5 and 2 percent of the weight of the base oil. Exceeding this proportion exerts an unfavorable influence on the stability of the oil. Moreover, oils treated by more than 1 percent coal oil have a very unpleasant odor.

It has now been discovered that the combination of heavy cycle gas oil and coal oil exerts a synergistic effect on the resistance of mineral oils to oxidation.

It has also been discovered that it is possible to add a large proportion of heavy cycle gas oil to a mineral oil to increase its aromatic character without impairing its stability, provided that a small quantity of coal oil is also added to the mineral oil.

The present invention therefore makes it possible to prepare mineral oils having both excellent resistance to oxidation and an aromatic character, two properties which, according to the previous proposals, were incompatible.

The process of the invention comprises adding to a mineral oil, for preference during refining, between 2 and 50 percent, or more particularly, between 3.5 and 25 percent by weight of heavy cycle gas oil, and between 0.1 and 5 percent or more particularly, between 0.2 and 1 percent coal oil as it is or modified by preliminary treatments.

The heavy cycle gas oil (H.C.G.O.) may have very variable characteristics according to the regulation of the cracking unit and the way in which it is separated by distilling from the other products derived from cracking. These characteristics are in general within the following limits:

|                                     |                                                              |
|-------------------------------------|--------------------------------------------------------------|
| Density at 15° C.                   | 0.990 to 1.100                                               |
| Viscosity at 98.9° C.<br>( 210° F.) | from 2 to 8 cst.                                             |
| Aniline Point                       | from 25° to 80° C.                                           |
| Distillation                        | between 180° and 660° C.<br>(at normal atmospheric pressure) |

The H.C.G.O. can be topped by distilling before being added to the base mineral oil. It is moreover advisable to dewax it before adding the base oil, if the final oil is required to have a cloud point (ASTM D 97.47) less than +5° C. For instance, by dewaxing a H.C.G.O. by the presently practiced processes, there is obtained with a yield of 80-85 percent, a product whose pour point is -15° C.; the final oil treated with the H.C.G.O. thus dewaxed has a cloud point of -40° C.

To increase the proportion of aromatics and heteroaromatics it is also possible to subject the H.C.G.O. whether or not dewaxed, before adding it to the mineral base oil, to a suitable treatment, such as extraction by a selective solvent (phenol for instance) so as to obtain a yield of extract or 80 to 95 percent, and better still from 90 to 95 percent.

It is an advantage to subject the H.C.G.O., whether or not dewaxed, or its solvent extract, before adding it to the oil, to mild acid treatment, such as treatment by 5 to 20 percent, and preferably 8 to 12 percent by weight of sulfuric acid of 98 percent strength; the acid tars are decanted hot (80° to 100° C.) then the acid raffinate is neutralized by an aqueous or alcoholic solution of a mineral base, washed with water and dried on a natural earth (silicoaluminate).

The coal oil, anthracene oil or chrysene oil, is obtained by distilling the tars derived from heat treatment of the coal. Its characteristics are generally within the following limits:

|                            |                 |
|----------------------------|-----------------|
| Density at 15° C.          | 1.000 to 1.200  |
| Flash Point (open vessel)  | 120° to 200° C. |
| Refractive index at 60° C. | 1.630 to 1.670  |
| Freezing Point             | -50° to +30° C. |
| sulfur                     | 0.3 to 0.9 %    |
| Nitrogen                   | 0.6 to 1%       |
| C/H (atomic ratio)         | 1.35 to 1.65    |

Particularly interesting results are obtained with those anthracene oils termed "pale at -5° C." or "pale at 0° C."

The coal oil may also undergo various classical treatments for purification before being added to the base mineral oil.

The H.C.G.O. and the coal oil, whether or not treated as mentioned above, may be added to the base oil to be improved, for preference before a finishing treatment with natural or activated earth, or better still with hydrogen. Alternatively, the H.C.G.O., the coal oil, as they are or having undergone one or more of the treatments mentioned above, and the base oil to be improved are subjected separately, or mixed in pairs or all together, to a finishing treatment (with natural or activated earth, or better still hydrogen) before mixing them.

The treatment with hydrogen can take in the presence of a hydrotreatment catalyst under the following ranges of conditions:

|                                                           |                                  |
|-----------------------------------------------------------|----------------------------------|
| Temperature (°C.)                                         | 200-300, more preferably 210-280 |
| Pressure (bars)                                           | 30-80, more preferably 40-70     |
| Space Velocity (Vols. feedstock/Vol. catalyst/hour)       | 0.3-2.0, more preferably 0.8-1.2 |
| Volumes H <sub>2</sub> (reduced to N.T.P.)/Vol. feedstock | 100-400, more preferably 125-250 |

The hydrotreatment catalyst may be any catalyst suitable for mild hydrogenation—for example, oxides and/or sulfides of cobalt, molybdenum, nickel or tin, among others, and the catalyst may be disposed on a supporting material such as silica or alumina.

It is possible, according to the aromatic nature of the raffinate and the quantities of H.C.G.O. and coal oil added, to

prepare oils which meet different operational requirements. In particular, it is possible to obtain exceptionally stable oils having an average aromatic character, or highly aromatic oils possessing sufficient stability.

A number of mineral oils will now be described by way of illustration only, some of the mineral oils being nonlimitative exemplary embodiments in accordance with the invention and the others, which are not in accordance with the invention, being described by way of comparison.

### EXAMPLE 1

#### Preparation of stable oils with medium aromatic character

A 330-410° C. light distillate derived from Tijuana crude was refined by solvent extraction with phenol so as to obtain a raffinate having a viscosity gravity constant (VGC) equal to 0.822, the yield of raffinate being 55 percent by volume. The parameter VGC is well known in the art, and is defined, for example, on page 82 of "ABC du Graissage," a publication of the Institut Francais du Petrole.

There was added to the light raffinate thus obtained (raffinate I) in various hereinafter-disclosed proportions, a H.C.G.O. having the characteristics hereinbefore referred to, and a coal oil (an anthracenic oil termed "pale at 0° C."), the characteristics of these components being as tabulated in table

(Volume of hydrogen)/Volume of oil) = 150  
(volumes referred to normal conditions of temperature and pressure).

The resistance to oxidation of the various oils thus prepared was investigated the so-called "BBC" (Brown Boveri Company) test which consists of heating to 110° C., 1,000 cc. oil in a copper pot in the presence of a cotton thread. After 72 hours and 168 hours, respectively, the NPA color (ASTM D 155) and the acid number (ASTM D 947) of the oil are determined, and also the quantity of deposits and the percentage of loss of resistance of the cotton thread. After 168 hours the dielectric losses are also measured and given as the tangent of the angle of loss of the tested oil.

To determine the proportion of aromatic carbon, the ndM method is used (refractive index-density-molecular mass) giving the proportion of aromatic carbon as a function of these three parameters. The Brandes method furnishes the same results by infrared investigation. The absorption of liberated gas is found by the Pirelli method. This consists of measuring, under well-defined conditions (16 kv.-300 minutes-80° C.) the tendency of the oil to absorb or desorb a gas (either hydrogen or nitrogen) with which the oil has previously been saturated.

A satisfactory oil must be able to absorb gas. Under the conditions stated above, figures in the region of 1.2 cc. hydrogen

TABLE II

| Oil composition                                                   | A          | B      | C                          | D      | E                          | F      | G                      | H                  |
|-------------------------------------------------------------------|------------|--------|----------------------------|--------|----------------------------|--------|------------------------|--------------------|
| Base Oil, Raffinate I                                             | 100        | 100    | 100                        | 100    | 100                        | 100    | 100                    | 100                |
| H.C.G.O. (wt. percent)                                            | 4          | 3.6    | 0.4                        | 12     | 12                         | 0.4    | 0.5                    | 1                  |
| Anthracene oil (wt. percent)                                      |            |        |                            |        |                            |        | 5.5                    | 6                  |
| Aromatic carbons (percent by ndM method)                          | 5          | 5.5    | 6                          | 7.5    | 8                          |        |                        | 4                  |
| Absorption of gases of hydrogen (Pirelli method) cm. <sup>3</sup> | 0.8        | 0.8    | 0.85                       | 1.2    | 1.2                        | 0.8    | 0.8                    | 1.1                |
| BBC test—                                                         |            |        |                            |        |                            |        |                        |                    |
| 72 hours:                                                         |            |        |                            |        |                            |        |                        |                    |
| Colour (NPA)                                                      | 4          | 2      | 2                          | 2      | 2                          | 1.5    | 2.5                    | 3                  |
| Acid number, mg.                                                  | 0.140      | 0.040  | 0.070                      | 0.050  | 0.030                      | 0.012  | 0.050                  | 0.075              |
| KOH/g.                                                            |            |        |                            |        |                            |        |                        |                    |
| Deposits, percent                                                 | 0.024      | 0.010  | 0.007                      | 0.015  | 0                          | 0.007  | 0.017                  | 0.020              |
| Percent loss of resistance of cotton thread.                      | 0          | 1      | 0                          | 0      | 0                          | 0      | 0                      | 0                  |
| 168 hours:                                                        |            |        |                            |        |                            |        |                        |                    |
| Colour (NPA)                                                      | 5          | 4      | 3                          | 4.5    | 3.5                        | 3.5    | 3                      | 3.5                |
| Acid number, mg.                                                  | 0.250      | 0.09   | 0.07                       | 0.14   | 0.04                       | 0.098  | 0.112                  | 0.15               |
| KOH/g.                                                            |            |        |                            |        |                            |        |                        |                    |
| Deposits, percent                                                 | 0.078      | 0.030  | 0.020                      | 0.040  | 0.002                      | 0.017  | 0.034                  | 0.045              |
| Percent loss of strength of cotton thread.                        | 20         | 25     | 22                         | 20     | 20                         | 17     | 0                      | 20                 |
| Tangent of angle of loss.                                         | 0.2680     | 0.0180 | 0.0105                     | 0.0300 | 0.0170                     | 0.0700 | 0.0175                 | 0.0250             |
| Remarks on overall characteristics and performance.               | Very poor. | Good.  | Excellent compared with B. | Good   | Excellent compared with D. | Poor   | Good, but strong smell | Very strong smell. |

I.

TABLE I

| Property                                | H.C.G.O. | Anthracene Oil |
|-----------------------------------------|----------|----------------|
| Density at 15° C.                       | 0.990    | 1.08           |
| Sulfur wt%                              | 2.23     | 0.54           |
| Nitrogen wt%                            | 0.08     | 0.81           |
| Flash Point, open vessel, °C.           | 142      | 128            |
| Viscosity at 98.9° C.<br>(210° F.) cst. | 2.96     | 2.64           |
| Pour Point °C.                          | -6       | -15            |

The mixtures thus prepared and, for the purpose of comparison, without added H.C.G.O. and oil raffinate, were subjected to a finishing treatment consisting of hydrogenation under the following conditions:

Cobalt molybdate on alumina catalyst (3.5% CoO and 12.5% MoO<sub>3</sub>)

Temperature: about 250° C.

Pressure: 60 bars

Space Velocity—(volume of oil per hour)/(volume of catalyst) = 1

are satisfactory. Nevertheless, certain users require higher absorption figures. The results obtained are given in table II, wherein the different oils bear the references A to H.

The oil C in accordance with the invention, with the simultaneous addition of H.C.G.O. and anthracene oil, is characterized by exceptional stability. It is found that this oil is more stable than oils B and G which contain respectively the optimum quantity of H.C.G.O. by itself and the anthracene oil by itself. The oil G has the further drawback of being evil smelling.

Oil E, which is also in accordance with the invention, has both excellent stability and gas-absorbing properties. Oil D has the same capacity for absorption but does not contain anthracene oil and is less stable than Oil E.

### EXAMPLE 2

#### Preparation of more highly aromatic oils with good stability

A light distillate derived from Tijuana crude was refined by phenol treatment so as to obtain a raffinate having a viscosity gravity constant equal to 0.832, the yield of raffinate being 65 percent by volume.

Then, under the conditions described in the previous example, and with a H.C.G.O. and a coal oil of similar nature, there were prepared with this raffinate (raffinate II) the oils referred to by the letters I to N, whose characteristics are given in table III.

TABLE III

| Oil composition                                               | I         | J      | K                          | L      | M                                                 | N                  |
|---------------------------------------------------------------|-----------|--------|----------------------------|--------|---------------------------------------------------|--------------------|
| Base oil, Raffinate II                                        | 100       | 100    | 100                        | 100    | 100                                               | 100                |
| H.C.G.O. (wt. percent)                                        |           | 4      | 3.6                        | 12     | 12                                                |                    |
| Anthracene oil (wt. percent)                                  |           |        | 0.4                        |        | 0.4                                               | 4                  |
| Aromatic carbon (percent, ndM method)                         | 11        | 12     | 12.5                       | 15     | 15.5                                              | 13.6               |
| Gas absorption (Pirelli method), cm. <sup>3</sup> of hydrogen | 1.4       | 1.45   | 1.45                       | 1.8    | 1.8                                               | 1.55               |
| BBC test—                                                     |           |        |                            |        |                                                   |                    |
| 72 hours:                                                     |           |        |                            |        |                                                   |                    |
| Colour (NPA)                                                  | 4         | 3      | 2                          | 4      | 2.5                                               | 3                  |
| Acid number, mg. KOH/g.                                       | 0.180     | 0.06   | 0.035                      | 0.084  | 0.040                                             | 0.085              |
| Deposits, percent                                             | 0.030     | 0.015  | 0.005                      | 0.006  | 0                                                 | 0.015              |
| Loss of strength of cotton thread                             | 0         | 0      | 0                          | 2      | 0                                                 | 0                  |
| 168 hours:                                                    |           |        |                            |        |                                                   |                    |
| Colour (NPA)                                                  | 5         | 4      | 3.5                        | 5      | 4                                                 | 6                  |
| Acid number, mg. KOH/g.                                       | 0.350     | 0.09   | 0.06                       | 0.13   | 0.07                                              | 0.18               |
| Deposition, percent                                           | 0.120     | 0.035  | 0.015                      | 0.050  | 0.006                                             | 0.080              |
| Loss of strength of cotton thread                             | 20        | 27     | 19                         | 26     | 11                                                | 15                 |
| Tangent of angle of loss (90° C.)                             | 0.3560    | 0.0300 | 0.0170                     | 0.0430 | 0.0300                                            | 0.0420             |
| Remarks on overall characteristics and performance.           | Very poor | Good   | Excellent compared with J. | Good   | Excellent compared with L. Note high aromaticity. | Very strong odour. |

The oils K and M of the invention, with the addition of H.C.G.O. and anthracene oil, display exceptional gas-absorbing properties and excellent stabilities compared with the oils J, N, and L, and clearly demonstrate the synergistic interaction of the H.C.G.O. and the anthracene oils, despite the fact that comparable proportions of aromatic compounds are present in many cases.

The present invention has been described by way of explanation but in no way restrictively. Any useful modifications may be made to it without departing from its scope as defined by the appended claims.

We claim:

1. A method of making an oxygen stable oil composition which comprises adding to a light straight run distillate oil from which the aromatics have been removed by solvent extraction from 2 to 50 wt. percent of heavy cycle gas oil (H.C.G.O.) and from about 0.2 to 1.0 wt. percent of coal oil, the weight percentages being based on the weight of the base oil.

2. A method according to claim 1 in which the H.C.G.O. has the following properties:

|                          |                                       |
|--------------------------|---------------------------------------|
| Density at 15° C.        | 0.990 to 1.100                        |
| Viscosity at 98.9° C.    | 2 to 8 cst.                           |
| Aniline point            | 25° to 80° C.                         |
| Distillation range (°C.) | 180 to 660<br>(reduced to 760 mm. Hg) |

3. A method according to claim 1 in which the H.C.G.O. has been dewaxed.

4. A method according to claim 1 in which the H.C.G.O. has been enriched in aromatic compounds by the use of a solvent extraction process.

5. A method according to claim 1 in which the H.C.G.O. has been topped by distillation.

6. A method according to claim 1 in which the H.C.G.O. has been subjected to an acid treatment.

7. A method according to claim 1 in which the H.C.G.O. forms the 3.5 to 25 wt. percent relative to the base oil.

8. A method according to claim 1 in which the coal oil has the following properties:

|                            |                 |
|----------------------------|-----------------|
| Density at 15° C.          | 1.00 to 1.20    |
| Flash point (open vessel)  | 120° to 200° C. |
| Refractive Index at 60° C. | 1.63 to 1.67    |
| Pour Point (°C.)           | -50 to +30      |
| Sulfur (wt.%)              | 0.3 to 0.9      |
| Nitrogen (wt.%)            | 0.6 to 1.0      |
| C/H atomic ratio           | 1.35 to 1.65    |

9. A method according to claim 8 in which the coal oil has been selected from the anthracene oils known as "pale at -5°

C." and "pale at 0° C."

20 10. A method according to claim 1 in which the base oil is a raffinate derived from a solvent extraction process.

11. A method according to claim 1 in which the base oil, H.C.G.O. and coal oil are subjected to a refining process in any combination, the refining process comprising contact with a natural earth or hydrotreatment.

25 12. A stable mineral oil made by a process in accordance with claim 1.

13. A stable mineral oil comprising a base oil of low aromatic content, from 2 to 50 wt. percent of heavy cycle gas oil and 0.2 to 1.0 wt. percent of coal oil, the heavy cycle gas oil having the following properties:

|                       |                                            |
|-----------------------|--------------------------------------------|
| Density at 15° C.     | 0.990 to 1.100                             |
| Viscosity at 98.9° C. | 2 to 8 cst.                                |
| Aniline Point         | 25° to 80° C.                              |
| Distillation range    | 180° to 660° C.<br>(reduced to 760 mm. Hg) |

and the coal oil having the following properties:

|                            |                 |
|----------------------------|-----------------|
| Density at 15° C.          | 1.00 to 1.20    |
| Flash Point (open vessel)  | 120° to 200° C. |
| Refractive Index at 60° C. | 1.63 to 1.67    |
| Pour Point (°C.)           | -50 to +30      |
| Sulfur (wt.%)              | 0.3 to 0.9      |
| Nitrogen (wt.%)            | 0.6 to 1.0      |
| C/H atomic ratio           | 1.35 to 1.65    |

40 14. A stable mineral oil according to claim 13 in which at least one of the base oil, heavy cycle gas oil and coal oil has been hydrotreated, in any combination with the other oils.

50 15. A stable mineral oil according to claim 14 in which the heavy cycle gas oil has been dewaxed.

16. A stable mineral oil according to claim 15 in which the heavy cycle gas oil is a dewaxed solvent extract of a topped heavy cycle gas oil fraction.

55 17. A stable mineral oil according to claim 16 in which the base oil is a mineral oil of relatively low aromatic content and the heavy cycle gas oil is a dewaxed solvent extract of an acid-treated, topped heavy cycle gas oil fraction.

60 18. A concentrate for stabilizing mineral oils to oxygen which consists essentially of about 28 to 99.8 wt. percent heavy cycle gas oil (H.C.G.O.) and 72 to 0.2 wt. percent coal oil.

65 19. A method as claimed in claim 1 wherein said composition is more stable than one made solely from said distillate oil and 2 to 50 wt. percent of said heavy cycle gas oil or one made solely from said distillate oil and 0.2 to 1.0 wt. percent of said coal oil.

\* \* \* \* \*